

## UNITED STATES PATENT OFFICE

1,974,477

## COATING FOR STEREO TYPE MATRICES

Louis G. Walters, New York, N. Y., assignor to  
 Electrographic Corporation, New York, N. Y.,  
 a corporation of Delaware

No Drawing. Application June 15, 1933,  
 Serial No. 675,971

6 Claims. (Cl. 91—68)

The present invention relates to a coating for the facing surface of a stereotype mat.

Stereotype mats are a special type of paper board and are sufficiently plastic to receive impressions from printing faces when the matrix board is pressed under substantial pressure against type or other printing faces. The impressed matrix board is then used as a mold face against which molten type metal is poured to form a stereotype printing plate. The texture of the surface of the matrix board is relatively coarse and does not produce a smooth printing surface. Furthermore, the fibrous material of which the matrix board is composed tends to burn out when subjected to a number of casts from hot type metal.

The present invention overcomes the difficulties of the known prior art by providing a surface coating on the matrix board, which coating will mold into the finest lines on half tones or type and is of such texture that the coating molds as a smooth surface against the smooth type face.

Furthermore, my new coating is of such material as to withstand the heat of molten type metal so that a number of casts may be made from a single matrix board.

Coatings for matrix board have heretofore been suggested but these coatings have been unsuccessful because of materials used in the coating producing undesirable and deleterious effects. It has been proposed to use binders in coatings which binders melt when subjected to heat and which binders tend to gasify when subjected to the heat of molten type metal. Such binders introduce several difficulties. It is customary to heat the type or plates from which the stereotype mat is made and coatings having binders which melt tend to stick to the heated type. Where such mats are used against cold type, the chief difficulty is postponed until the melted type metal strikes the mat when the binder first melts and then gasifies, thereby producing a very rough surface. The coating also tends to stick to the molded stereotype plate and thus the matrix is destroyed when the matrix board is removed from the stereotype plate.

A still further and important attribute of a coating for a stereotype plate is that the coating must be extremely flexible and rubber-like at the time when the matrix board is forced under pressure against the type and printing faces. The coating must not shrink to any substantial extent when it dries out, otherwise it will distort the matrix impressions. Unless the coating is flexible and capable of stretching, it will

break over the edges of the type faces and form small cracks. When the molten type metal is cast against a cracked matrix, the metal flows into these cracks and interlocks with the coating. This tears away a part of the matrix surface when the matrix board is removed from the cast plate.

The present invention overcomes the difficulties of the known prior art and in actual use has demonstrated that it is a practical commercial product comprising a substantial improvement in the art.

The present coating comprises the use of colloidal-graphited water (sold under the trade name of "Aquadag"), mixed with distilled water and potato starch. The preferred formula is ten ounces of Aquadag plus four ounces of potato starch, added to one gallon of luke warm distilled water. The materials are thoroughly mixed and when so mixed will stand for substantial lengths of time without any change or deterioration. Preferably, the coating material is heated to luke warm temperature or approximately 100° F. and then is applied to one face of the matrix board. The coating may be applied by brushing the surface of the board with the liquid coating or by spraying the coating on the board in the usual manner of spraying paint materials.

Preferably, two coats of the material are applied to the matrix board. The first coat acts as a priming coat and soaks into the matrix board. In a seven ply matrix board, the coating appears to soak through substantially three plies. This first coat is permitted to dry and then a second coat is laid on in the same manner as the first coat. The second coat forms a perfect bond with the first coat and lays substantially entirely upon the surface so as to form a surface layer of graphite and potato starch after the carrying medium, namely, the water, has been dried out. Other starches have been tried such as corn starch, or a wheat starch, but potato starch seems to be the most satisfactory in that it is finer and lighter than other forms of starch. It remains in solution and also produces a very fine grain coating on the surface of the matrix board when the coating has dried.

The coated sheet may be used as a so-called dry mat, or as a wet mat. Preferably, it is used as a wet mat and when so used, it is desirable to moisten the back of each sheet with a sponge soaked in water. Then, the sheets are piled back to back and face to face, and after fifteen minutes time are ready for use. The surface coat at this time is of a rubbery consistency and will

- bend and stretch without breaking. The matrix board is applied with coated side toward the type or plates from which the mold is to be made. The type or plates are preferably heated to about 150° F. and the matrix board is pressed against the printing faces with a substantially heavy pressure sufficient to impress the type faces into the coated surface. This pressure may be quickly released and then the type with the matrix board resting thereon may be moved to a steam table and subjected to lighter pressure for two or three minutes which is sufficient time to completely drive out the moisture from the mat and the mat is then ready for use as a stereotyping mat.
- This new coating does not shrink seriously when drying and does not pull or produce double impressions as is the case where the prior art coated mats are pressed and the pressure released and re-applied.
- The matrix board is now ready for use, and may be used with higher temperatures than other matrix boards heretofore used in the art. Preferably, applicant's matrix is used with type metal heated to about 800° F. and even with this high temperature, many stereotype plates may be made from a single matrix without burning or destroying the matrix.
- Applicant's matrix requires no face treatment as is common in the art of stereotyping. Usually, stereotype matrices are coated with French chalk or zinc stearate or other face treatment compounds. In this new mat, the face as it leaves the printing type is ready for immediate use without further treatment of any kind.
- The coating on the novel mat herein described adheres very tightly to the face of the matrix board and does not tend to chip or peel off. When the mat has been pressed against the type, the impression surfaces present a bright polished appearance which is retained during the subsequent use of the mat.
- What I claim is:—
1. The process of preparing a matrix board for stereotyping comprising applying to a surface of said board as a coating a solution of colloidal-graphited water and starch suspended in water, and drying the coated surface to leave thereon a coating of very finely divided graphite and starch particles.
  2. The process of preparing a matrix board for stereotyping comprising applying a priming coat to a surface of said matrix board of a solution of colloidal-graphited water and starch suspended in water; permitting the priming coat to soak into said board; drying the priming coat; applying a cover coat of said graphite, starch, and water solution to form a layer of finely divided graphite and starch covering a surface of said board; and drying off the excess water from said cover coating.
  3. An article of manufacture comprising a matrix board for stereotyping having a surface thereof covered with a coating of very finely divided graphite deposited from a colloidal graphited water solution and starch particles.
  4. An article of manufacture comprising a matrix board for stereotyping having a face thereof impregnated with a water solution of very finely divided graphite and starch, and with a layer of impregnating material forming a covering surface of graphite and starch overlying a face of the said board.
  5. An article of manufacture comprising a matrix board for stereotyping having a surface thereof covered with a coating comprising a mechanical mixture of very finely divided graphite and potato starch, said coating being of sufficient thickness and depth to completely cover the fibers of said board whereby the coating receives the impression when said board is used for stereotype molding.
  6. An article of manufacture comprising a matrix board for stereotyping having a surface thereof coated with finely divided graphite deposited from a colloidal graphited water solution and potato starch, the graphite and potato starch being substantially in the proportions by weight of ten percent wet graphite with four percent dry starch.
- LOUIS G. WALTERS. 120
- 50 125
- 55 130
- 60 135
- 65 140
- 70 145
- 75 150